

June 12, 1934.

L. G. S. BROOKER

1,962,123

PHOTOGRAPHIC EMULSION CONTAINING DIBENZOXACARBOCYANINES

Filed Feb. 20, 1932

Fig.1.

2:2'-Dimethyl-3:4:5':4'-dibenzoxacarbocyanine bromide.



Fig.2.

2:2'-Diethyl-3:4:5':4'-dibenzoxacarbocyanine bromide.



Inventor:

Leslie G. S. Brooker,

Attorney:

By

Daniel J. Mayne

Attorneys.

## UNITED STATES PATENT OFFICE

1,962,123

PHOTOGRAPHIC EMULSION CONTAINING  
DIBENZOXACARBOCYANINESLeslie G. S. Brooker, Rochester, N. Y., assignor to  
Eastman Kodak Company, Rochester, N. Y., a  
corporation of New York

Application February 20, 1932, Serial No. 594,381

6 Claims. (Cl. 95—7)

This invention relates to a photographic emulsion sensitized by a new class of photographic sensitizing dyes, and more particularly to gelatino-silver-halide emulsions sensitized with a new 5 class of dyes known as the dibenzoxacarbocyanines and to photographic elements comprising such an emulsion.

It has been known for some time in the photographic art that in order to render photographic 10 emulsions, such as gelatino-silver-halide emulsions, sensitive to substantially all of the visible rays of the spectrum, it is necessary to treat the emulsions, either by overcoating or by admixture with the emulsions themselves, with a compound 15 which extends or enhances the sensitivity of the emulsions to light beyond their natural sensitivity. Many dyes suitable for this purpose have been 20 previously described in the literature, such for instance as pseudocyanine, sensitol red, kryptocyanine, thiocarbocyanine, and others. Additional ones have also been described in my previously filed co-pending applications, such for instance as the naphthocarbocyanines described in my 25 U. S. Patent No. 1,846,300 of Feb. 23, 1932 and my application Serial No. 435,105 filed March 12, 1930. The dibenzoxacarbocyanines described in the instant application were likewise described in my U. S. Patent No. 1,846,300 of Feb. 23, 1932, in which it was related that instead of employing 30 a methylnaphthothiazole as the starting material for producing the dibenzocarbocyanine, one could replace the sulphur in the thiazole by oxygen and produce a dibenzoxacarbocyanine by using the methylnaphthoxazole as the starting material. 35 These dibenzoxacarbocyanines sensitize a gelatino-silver-halide emulsion containing them to the yellow-green portion of the spectrum, contributing a maximum sensitivity at approximately 5550 Angstrom units.

It is an object, therefore, of this invention to provide a photographic emulsion such as gelatino-silver-halide emulsion, which contains a new 40 sensitizing dye belonging to the class of dibenzoxacarbocyanines and to prepare photographic elements having a transparent support coated with such an emulsion. Other objects will occur to those skilled in the art upon a further perusal of this specification.

The compound known as 2-methyl-β-naph-

thoxazole, for instance, was first described, together with its method of preparation, by Böttcher (Ber., 1883, 16, 1933). A somewhat different method of preparing this base was later described by Michel & Grandmougin (Ber., 1892, 25, 3429). 55 The structure of the 2-methyl-β-naphthoxazole is as follows:



60

65

The numbering given is that used in Richter's "Lexikon der Kohlenstoff Verbindungen" and also in "Chemical Abstracts." The 1-methyl-α-naphthoxazole may be prepared from 2-amino-1-naphthol in a manner similar to that described by Michel and Grandmougin (loc. cit.) for the isomeric 2-methyl-β-naphthoxazole. 70

This base will yield dibenzoxacarbocyanine dyes, the formation of which probably takes place 75 as follows: first, the base is converted into a suitable alkyl quaternary salt, such as the methoxy etho-p-toluenesulfonate or the methiodide or ethiodide, by heating the base with a suitable substance such as methyl p-toluenesulfonate or 80 methyl iodide under appropriate conditions, for instance,



where R is an alkyl group such as methyl or ethyl, 95 and X is a suitable acidic radical, such as p-toluenesulfonate or iodide.

This quaternary salt, for instance, 2-methyl-β-naphthoxazole metho-para-toluenesulfonate (2 mols.) is then heated with ethyl orthoformate 100

(1 mol.) in the presence of anhydrous pyridine whereupon the dye is formed. The reaction may be represented as follows:

Examples of specific methods by which these dyes may be prepared are as follows, but it will of course be understood that these are not limit-



25 In practice a better yield of dye is obtained if an excess of ethyl orthoformate is employed over that theoretically necessary. Other ortho-esters of formic acid, such as trimethyl orthoformate, may, of course, be used. It is desirable to number the dye molecule in the above fashion in order that this numbering will be in accord with that given to the sulphur containing dye named, for instance, in my application Serial No. 337,177. The final name for a dye of this type therefore becomes 2,2'-dialkyl-3:4:3':4'-dibenzoaxacarbo-cyanine salt. In the above formulae, R may be similar or dissimilar alkyl radicals depending upon whether the naphthoxazole quaternary salt contains only the one alkyl radical or whether two portions of the salt are employed each having a different alkyl radical.

After the formation of the dye, it may be isolated and purified by ordinary chemical methods, or it may be converted into another salt, usually a less soluble one, by double decomposition in the ordinary fashion. For instance the p-toluenesulfonate of a dye may be converted into a bromide by treatment, in solution, with a soluble bromide, such as sodium bromide. The acid radical finally employed may be one such as a halide, perchlorate, nitrate, acetate, p-toluenesulfonate or in fact any salt forming acid radical which will not greatly decrease or destroy the sensitizing properties of the dye. X in the above formulae of the carbocyanines may represent any of these acid radicals.

In the dyes the two naphthoxazole nuclei are linked together by a chain comprising three carbon atoms. Since the  $=\text{CH}-$  group is called the methenyl group, the chain  $=\text{CH}-\text{CH}=\text{CH}-$  may be called a trimethenyl chain. Cyanine dyes containing this trimethenyl chain are commonly called carbocyanine dyes.

The diagrammatic spectrograms constituting the accompanying drawing illustrate the region of the spectrum to which the specific dyes herein disclosed will sensitize a gelatino-silver-halide emulsion and the extent of the sensitization at various wave lengths. The figures of the drawing and the dyes, the sensitizing properties of which they illustrate, are as follows:

Fig. 1. 2:2'-dimethyl-3:4:3':4'-dibenzoxacarbocyanine bromide.

Fig. 2. 2:2'-diethyl-3:4:3':dibenzoaxacarbo-cyanine bromide.

ing but merely illustrating the manner of effect- 100  
ing the broad principles of my invention.

*Example I—2:2'-dimethyl-3:4:3':4' - dibenzoxa-carbocyanine bromide*

6.1 g. 2-methyl- $\beta$ -naphthoxazole is heated with 6.2 g. methyl p-toluenesulfonate for 6 hours at about 160° C. During a further 15 hours heating at 130-140° C. the product solidifies to a brownish solid. The product, substantially 2-methyl  $\beta$ -naphthoxazole metho-p-toluenesulfonate, is boiled under reflux with anhydrous pyridine (40 cc.) and ethyl orthoformate (5.5 cc., 100% excess). A reddish orange color forms rapidly and refluxing is continued for 45 minutes. A hot solution of excess of potassium bromide (20 g.) in water (100 cc.) is added to the reaction mixture, and the dye is rapidly precipitated as the bromide. The crude dye may be freed from impurities by boiling it successively with water and then with acetone, and then recrystallizing it from methyl alcohol, whereupon it is obtained as a mass of red silky needles which give an orange solution in the solvent. 110 115 120

*Example II*—2:2' - diethyl-3:4:3':4' - dibenzoxa- 125  
carbocyanine bromide

9.15 g. 2-methyl- $\beta$ -naphthoxazole is condensed with 10 g. ethyl p-toluenesulfonate by heating for 6 hours at 160°-180° C. and for 15 hours at 130°-140° C. The crude quaternary salt as thus obtained forms a very viscous yellowish-brown liquid.

The crude product obtained above, substantially 2-methyl- $\beta$ -naphthoxazole etho p-toluene-sulfonate may be used without purification. It is refluxed for 45 minutes with anhydrous pyridine (30 cc.) and ethyl orthoformate (8.2 cc., 100% excess). The dye is then precipitated as the bromide by adding an excess of a warm solution of potassium bromide (20 g.) in water (100 cc.). After filtering, the dye may be washed with water and then with hot acetone and finally recrystallized from methyl alcohol, in which it gives an orange solution. It is obtained as reddish needles. 135 143 145

In the same manner that the 3:4:3':4' dibenzox-carbocyanine is prepared, one may prepare the 5:6:5':6'-dibenzoxacarbocyanine, if one were to start with the 1-methyl-alpha-naphthoxazole instead of the 2-methyl-*o*-naph-

thoxazole as above described. The structure of the base is given below, as well as that of an oxacarbocyanine dye derived from it.

5

1-methyl- $\alpha$ -naphthoxazole

10



2,2'-dialkyl-5:6:5':6'-dibenzoxacarbocyanine salt

15

20

80

85

90

95

25 The numbering is that used in my application where the corresponding sulfur-containing compounds were used, namely No. 337,177.

Since the preparation of 1-methyl- $\alpha$ -naphthoxazole is not described in the literature it 30 will be given here.

2-nitro-1-naphthol is first prepared (see, for instance, Hodgson & Kilner, J. C. S. 1924, 125, 807). This compound is then reduced to the corresponding 2-amino-1-naphthol, using tin and hydrochloric acid as recommended by 35 Liebermann & Dittler (Ber., 1874, 7, 240; Liebermann, Ann., 1876, 183, 246). The hydrochloride of the base is then heated with acetic acid and sodium acetate for several hours in a similar 40 fashion to that prescribed for the preparation of 2-methyl- $\beta$ -naphthoxazole by Michel & Grandmougin (Ber., 1892, 25, 3429). The excess of acetic acid is then slowly distilled off and the residue is finally distilled in vacuum, using 45 an oil bath to heat the reaction flask. The base distills over and is purified by dissolving the distillate in ligroin, allowing a solid impurity to crystallize out first, and then isolating the base from the mother liquor. The 1-methyl- $\alpha$ -naphthoxazole is obtained as a low melting solid.

50 For the preparation of the dyes the base is converted into a quaternary salt such as the methyl p-toluenesulfonate or the ethiodide in the usual way. The quaternary salt is then 55 condensed with ethyl orthoformate in the presence of anhydrous pyridine as described for the isomeric dyes derived from 2-methyl- $\beta$ -naphthoxazole.

### Example III

60 1 part of 1-methyl- $\alpha$ -naphthoxazole is heated on a steam bath with 1.05 parts of methyl p-toluenesulfonate for several hours. Addition is rapid and the quaternary salt, 1-methyl- $\alpha$ -naphthoxazole metho p-toluenesulfonate sets to a mass of crystals. This is then refluxed with 65 25 parts of anhydrous pyridine and 1.6 parts of ethyl orthoformate (300% excess of the latter);— the yield is improved by taking an excess of the 70 ester). Within a few minutes the dye begins to separate, the p-toluenesulfonate of the dye being very sparingly soluble in pyridine, hot or cold. After 30 minutes refluxing, the reaction mixture is allowed to cool, and the dye is then 75 filtered off and washed with cold pyridine and

then dried. The yield is about 1.3 parts. This dye is 2,2'-dimethyl-5:6:5':6'-dibenzoxacarbocyanine p-toluenesulfonate.

The dye may be converted into the bromide by dissolving it in boiling methyl alcohol and adding an excess of an aqueous solution of an alkali bromide, such as potassium bromide, to the alcoholic solution. The bromide of the dye is almost insoluble in alcoholic-aqueous solution in the presence of a large excess of bromide ions and may be filtered off, washed with water, and then purified by recrystallization from ethyl or methyl alcohol. This dye is called 2,2-dimethyl-5:6:5':6'-dibenzoxacarbocyanine bromide. If potassium iodide is used in place of potassium bromide then the still less soluble dye iodide is formed. The bromide of the dye crystallizes from methyl alcohol as a felted mass of hair-like crystals, reddish-orange in color. The solution of the dye in the solvent named is orange.

### Example IV

If 1.1 parts of ethyl p-toluenesulfonate are used instead of the 1.05 parts of methyl p-toluenesulfonate used in the preceding example, and 100 the two components are heated on the steam bath for 24 hours, 1-methyl- $\alpha$ -naphthoxazole etho-p-toluenesulfonate is produced. This salt is condensed with ethyl orthoformate in boiling pyridine solution in the same manner described 105 in the preceding example, using 10 parts of pyridine and 1.6 parts of the ortho-ester. After 30 minutes refluxing the dye is precipitated from the deeply colored solution by adding thereto an excess of an aqueous solution of potassium iodide. 110 The dye is filtered off, washed with water and with acetone, and is purified by several recrystallizations from methyl alcohol, in which it gives an orange solution. The 2,2'-diethyl-5:6:5':6'-dibenzoxacarbocyanine iodide is obtained in 115 beautiful garnet-red crystals with a strong blue reflex.

The naphthalene nuclei in both the mu-methyl naphthoxazoles may be left unsubstituted or they 120 may be substituted.

In the preparation of emulsions containing these photographic sensitizers, it has been found that the dye may be dissolved in methyl alcohol and a volume of solution diluted with water and containing from 5 to 100 milligrams of dye added 125 to 1000 cc. of emulsion. While it may not be necessary to add some of the sensitizers in a large amount, it may be necessary to add others in amounts larger than those given above; generally about 10 to 20 milligrams is sufficient to obtain 130 the maximum sensitizing effect with a dye having good sensitizing power. The more powerful dyes, however, may require much less. The regulation or adoption of the most economical proportions will be apparent to those skilled in 135 the art upon observing the sensitizing power of the particular dye for the particular emulsion to be formed. The above examples are, therefore, illustrative and not to be understood as limiting the invention in any sense, as it will be 140 apparent that these dyes may be incorporated by other methods in many of the photographic emulsions customarily employed in the art, such for instance as by bathing the plate or film, upon 145 which the emulsion has been coated, in a solution of the dye in an appropriate solvent although this method of incorporating the dye in the emulsion is not preferred over that above described. Obviously the claims are all intended to cover any combination of these dyes with a 150

photographic emulsion whereby the dye exerts a sensitizing effect upon the emulsion.

What I claim is:

1. A photographic gelatino-silver-halide emulsion containing a dibenzoxacarbocyanine salt.
2. A photographic gelatino-silver-halide emulsion containing a dialkyl-dibenzoxacarbocyanine salt.
3. A photographic gelatino-silver-halide emulsion containing a dialkyl-dibenzoxacarbocyanine bromide.

4. A photographic gelatino-silver-halide emulsion containing a 2:2'-dialkyl-3:4:3':4'-dibenzoxacarbocyanine salt.

5. A photographic gelatino-silver-halide emulsion containing a 2:2'-dimethyl-3:4:3':4'-dibenzoxacarbocyanine bromide.

6. A photographic gelatino-silver-halide emulsion containing a 2:2'-dialkyl-3:4:3':4'-dibenzoxacarbocyanine bromide.

85

LESLIE G. S. BROOKER.

85

15 90

20 95

25 100

30 105

35 110

40 115

45 120

50 125

55 130

60 135

65 140

70 145

150